

(No Model.)

G. U. MEYER.  
SEAMLESS PLATED WIRE.

No. 441,886.

Patented Dec. 2, 1890.

Fig. 1.



Fig. 2.



Fig. 3.



Fig. 4.

16

WITNESSES:

Henry J. Miller  
Henry A. McLean

INVENTOR:

George U. Meyer  
By Joseph A. Miller, Co.  
Attest.

# UNITED STATES PATENT OFFICE.

GEORGE U. MEYER, OF PROVIDENCE, RHODE ISLAND.

## SEAMLESS PLATED WIRE.

SPECIFICATION forming part of Letters Patent No. 441,886, dated December 2, 1890.

Application filed September 9, 1890. Serial No. 364,460. (No specimens.)

*To all whom it may concern.*

Be it known that I, GEORGE U. MEYER, of Providence, in the county of Providence and State of Rhode Island, have invented a new 5 and useful Improvement in Seamless Plated Wire; and I hereby declare that the following is a full, clear, and exact description of the same, reference being had to the accompanying drawings, forming part of this specification.

This invention has reference to an improvement in the process for making ingots, consisting of a core of inferior metal and a seamless outer tube of superior or precious metal and 15 drawing or rolling these ingots into seamless plated wire.

The invention consists in cutting a disk from a sheet of plating metal, securing the disk to the end of the inferior metal forming 20 the core, drawing the disk over the core to form the ingot, and then drawing or rolling the ingot into wire.

In the manufacture of ingots for seamless plated wire a tube has heretofore been made 25 of the precious metal, which was placed over the core of inferior metal and secured to the same by the sweating or the soldering process to form the ingot from which the wire was drawn or rolled.

30 The object of this invention is to draw the tube from a flat sheet of metal at once over the core and secure the so-formed plating-tube to the core to form the ingot, or to roll or draw out the ingot into wire and secure 35 the seamless plating metal to the core of the wire at any step desired, subsequent to the drawing out of the wire.

Figure 1 is a sectional view of a core-piece, to one end of which a disk of plating metal 40 is secured by the screw-threaded draw-hook. Fig. 2 is a sectional view of a core-piece provided with a screw-threaded extension, forming a draw-bar, to which a disk of plating metal is secured. Fig. 3 is a perspective view 45 of the plating-disk, and Fig. 4 is a side view of a piece of seamless plated wire.

In the drawings, 7 indicates the disk of plating metal provided with the central hole 8. The disk of plating metal 7 is made 50 from a sheet of precious metal, when it is desired to secure the plating metal to the core by the sweating process. The disk may,

however, be made out of a sheet of what is known in the jewelers' art as "stock-plate"—that is, a plate of inferior metal plated with 55 precious metal.

In the preferred form indicated in the drawings the disk 7 is made up of a sheet of inferior metal plated on one side with a thin sheet of precious metal and on the other side 60 with a film of solder or metal that will flow at a lower temperature than the precious metal. In Figs. 1 and 2 the inferior metal is shown in section and indicated by the Fig. 9, the plate of precious metal shown by a heavy 65 line by the figure 10, and the surface plated with a solder or easier-flowing metal by the figure 11.

12 indicates the cylindrical core of inferior metal, 13 the screw-threaded extension 70 of the core, 14 the drawing-hook screw-threaded in the core 12, and 15 the nuts by which the plating-disk 7 is secured to the end of the core 12.

In carrying out my invention I cut from a 75 sheet of plating metal, consisting either of precious metal, of precious metal covered on the face toward the core with an easier-flowing metal, of inferior metal covered on one side with precious metal and on the other 80 with a metal fusing at a lower temperature than the precious metal, or from any other sheet of metal or composition of metals desired, a circular disk 7 of a diameter greater than the diameter of the core 12. This disk 85 I now secure to the end of the core 12, preferably by punching the hole 8 through the center of the disk and securing the disk by the extension 13, or the hook 14, and the nut 15; but the disk 7 may be secured to the end 90 of the core by solder in any other practical manner. I now draw the disk with the core through a series of holes in the draw-plate of an ordinary draw-bench used for drawing rods and wire. The disk enters the successive 95 holes, which, commencing with a hole but little smaller in diameter than the disk, gradually diminish in diameter, and is gradually drawn over the core until it covers the same, as is indicated in broken lines in Figs. 10 and 2.

In the preferred form I cut the disk from a sheet of metal composed of a sheet of inferior metal 9, plated on one side with the precious

metal 10 and on the opposite side with the easier-flowing metal or solder 11. I secure this disk to one end of the cylindrical core 12, draw the disk over the core, as above described, in a draw-bench, rolls, or by any other suitable means, to form the ingot, and then draw or roll the ingot into the wire 16. (Shown in Fig. 4.) This formed wire consists of a solid core and a seamless plating-tube of precious metal with a film of easier-flowing metal or solder between the core and the plating metal. It forms a solid rigid wire, which can be formed into any desired article for which plated wire is used, and, when formed into chain-links or other similar articles in which the ends of the wire are required to be soldered together, or to some other metal, by placing a little flux at the end or ends and heating the same sufficient to fuse the easier-flowing metal or solder, the parts will unite together by the internal solder, forming a strong and durable union.

It is evident that if required the core 12

may be a tube, so that when drawn out the wire will form a seamless plated tubular wire. 25

Having thus described my invention, I claim as new and desire to secure by Letters Patent—

1. The process herein described for making ingots for seamless plated wire, the same consisting in preparing a core of inferior metal, securing a disk of plating metal to one end of the core, and drawing, rolling, or forming the outer portion of the disk over the core, as described. 30

2. As a new article of manufacture, a seamless plated wire consisting of a core of inferior metal, a seamless plating of precious metal, and a film of easier-flowing metal or solder between the core and the plating metal, 4c as described. 35

GEORGE U. MEYER.

Witnesses:

J. A. MILLER, Jr.,

HENRY J. MILLER.